

SEPARATING PROTOACTINIUM WITH  
MANGANESE DIOXIDE

Glenn T. Seaborg, Chicago, Ill., John W. Gofman, Berkeley, Calif., and Raymond W. Stoughton, Oak Ridge, Tenn., assignors to the United States of America as represented by the United States Atomic Energy Commission

No Drawing. Application November 3, 1944  
Serial No. 561,837

## 8 Claims. (Cl. 23—14.5)

The invention relates to the preparation of masses and compositions of the isotope of uranium having a mass number of 233, said isotope being designated as  $_{92}\text{U}^{233}$  or  $\text{U}^{233}$ .

An object of the invention is to provide an improved method for preparing and isolating  $\text{Pa}^{233}$  and  $\text{U}^{233}$ .

Other objects and advantages of the invention will become apparent as the following detailed description progresses.

In this specification and the claims the name of the element is used to designate the element generically, either in its elemental state or combined in a compound, unless otherwise indicated by the sense in which it is used or by a specific designation such as "metal" or "elemental."

It is known that the bombardment of thorium with fast neutrons of energies above about 2 million electron volts (2 m. e. v.) results in a fission of the thorium.

We have discovered that the bombardment of thorium with neutrons having energies of below 1 million electron volts (1 m. e. v.) results not only in the production of  $\text{Pa}^{233}$  and ultimately of  $\text{U}^{233}$  through the prolonged decay of  $\text{Pa}^{233}$ , and further that  $\text{U}^{233}$  so produced undergoes fission with neutrons of such low energies as below 1 million electron volts (1 m. e. v.) and even with thermal neutrons. The production of  $\text{U}^{233}$  and/or  $\text{Pa}^{233}$  is thus complicated by the fact that  $\text{Pa}^{233}$  and/or  $\text{U}^{233}$  produced by neutron bombardment may be decomposed by fission under the same bombardment.

In accordance with the present invention we have provided a method of preparing  $\text{Pa}^{233}$  and  $\text{U}^{233}$  in substantial amounts and in concentrated form generally as a composition wherein  $\text{U}^{233} + \text{Pa}^{233}$  or the compounds thereof is the preponderant component of the composition and preferably as a composition containing not in excess of about 10 percent by weight of impurities. Further we have discovered that  $\text{U}^{233}$  may be effectively prepared as a concentrate by separating  $\text{Pa}^{233}$  from neutron irradiated thorium preferably by means of a carrier such as manganese dioxide and thereafter permitting the separated  $\text{Pa}^{233}$  to decay to  $\text{U}^{233}$ . In addition we have found that effective concentrates of these materials may be secured by treatment of neutron irradiated thorium which has been subjected to high intensity irradiation for a time sufficient to produce  $\text{Pa}^{233} + \text{U}^{233}$  in concentrations within a predetermined range.

The reaction of thorium with slow and moderately fast neutrons may be summarized as follows:



The fission products which are produced as a result of the fission of  $\text{U}^{233}$  with slow and moderately fast neutrons are, so far as we have been able to determine, the same as those produced by the fission of  $\text{U}^{235}$ . They consist of a large number of elements which generally fall into a light group with atomic numbers from 35 to 46 incl.

and a heavy group with atomic numbers from 51 to 60 incl., and which undergo beta decay. The fission products which have a half life of more than three days will remain in the reaction mass in substantial quantities at least one month after the termination of the reaction, and the removal or elimination of these products by our process is particularly advantageous. Among these products are: Sr, Y, Zr, Cb, Ru, Te, I, Xe, Cs, Ba, La, and Ce of a 20 day half life, and Ce of a 200 day half life.

10 In accordance with one embodiment of this invention, the mass of thorium is subjected to the action of neutrons, the majority of which have energies below 1 million electron volts, and the reaction of the neutrons with the thorium is terminated prior to the time when the neutrons are absorbed by the  $\text{U}^{233}$  at the same rate that they are absorbed by the  $\text{Th}^{232}$ . This limit is approximately when the weight ratio of  $\text{U}^{233}$  to unreacted  $\text{Th}^{232}$  is 1 to 100. In other words, the reaction of  $\text{Th}^{232}$  with neutrons should preferably be terminated prior to when the amount of  $\text{U}^{233}$  is approximately 1 percent of the amount of thorium present in the mass. When the reaction is terminated at or prior to this point there is also no danger during the reaction of a substantial decomposition of the  $\text{U}^{233}$  taking place by a nuclear self-sustaining chain reaction.

15 It is generally desirable to terminate the reaction of the neutrons with  $\text{Th}^{232}$  when the amount of  $\text{U}^{233} + \text{Pa}^{233}$  is much less than 1 percent of the unreacted amount of  $\text{Th}^{232}$  in order to reduce the amount of fission products and make it possible to isolate the  $\text{U}^{233}$  by ordinary chemical means without the use of large quantities of special materials such as refrigerating devices, radiation shields, special radiation resistant materials and the like. In order to reduce such special equipment to a minimum and at the same time have a practical amount of  $\text{U}^{233}$  and  $\text{Pa}^{233}$  for isolation by batch process, the reaction is terminated at a weight ratio of  $\text{U}^{233} + \text{Pa}^{233}$  to  $\text{Th}^{232}$  of not less than about 1 to 1 million and frequently between about 1 to 10,000, and 1 to 1,000.

20 The reaction of thorium either in metallic state or a compound such as an oxide or carbonate of thorium with neutrons to produce  $\text{Pa}^{233}$  and  $\text{U}^{233}$  may be carried out with neutrons from any suitable neutron source. Where the neutron source provides fast neutrons, the fast neutrons are slowed to neutrons having energies of below 1 million electron volts by interposing neutron slowing material between the fast neutrons and the thorium. Such neutron slowing materials include carbon-containing, deuterium-containing, or hydrogen-containing material such as graphite, paraffin, or deuterium oxide. Sufficient neutron slowing material is used so that at least a majority of the neutrons are slowed to energies of below about 1 million electron volts, since at higher energies there is very little production of  $\text{U}^{233}$  and considerable fission of the thorium. We may interpose the neutron slowing material between the fast neutrons and the thorium-containing mass, or we may admix neutron slowing material with the thorium. An intimate mixture of thorium with neutron slowing material may be readily obtained by using hydrated thorium compounds such as the compound  $\text{Th}(\text{OH})_4 \cdot \text{H}_2\text{O}$ . Since the slow neutron absorption cross section of thorium is some ten to forty times larger than that of hydrogen, we may suitably use a ratio as high as about two to four hydrogen atoms per thorium atom without losing any more than 10 percent of the neutrons as a result of absorption by hydrogen.

25 While neutrons obtained from any suitable source of high neutron output may be used, it is desirable to subject the thorium to neutrons from a high intensity source in order that suitable concentrations of  $\text{Pa}^{233}$  and  $\text{U}^{233}$  may be obtained in a reasonable length of time.

Preferably the thorium is subjected to slow neutrons from a source of neutrons capable of supplying at least  $5 \times 10^{17}$  neutrons per second to the thorium mass and where a relatively high concentration of  $U^{233} + Pa^{233}$  is desired should weigh no more than about 20 tons. Preferably this mass should be of such a thickness that at least 50 percent and preferably 75 percent or more of the neutrons supplied are absorbed. Such high neutron intensity may be obtained by subjecting thorium to the action of neutrons obtained by slowing down secondary neutrons obtained from a self-sustaining chain reaction of  $U^{233}$ ,  $U^{235}$  or  $94^{239}$  with neutrons.

By placing thorium adjacent to a neutron chain reacting mass comprising uranium and/or  $94^{239}$  in amount sufficient to establish a self-sustaining neutron chain reaction dispersed in a neutron slowing medium such as carbon or  $D_2O$ , between  $5 \times 10^{17}$  and  $10^{20}$  neutrons per second are supplied to the thorium and at least 50 to 75 percent are absorbed so that a ratio of  $U^{233} + Pa^{233}$  to  $Th^{232}$  of more than 1 to 1 million may be attained in a reasonable length of time, such as one to three months. In such a case the degree of bombardment desired may be completed before the preponderant amount of  $Pa^{233}$  formed has decayed to  $U^{233}$ .

The method of chemical separation here involved is based upon the initial separation and recovery of  $Pa^{233}$ , followed by conversion of the  $Pa^{233}$  to  $U^{233}$  and the subsequent separation of these two elements.

A suitable method which is particularly effective for isolating  $Pa^{233}$  and  $U^{233}$  described below is given by way of example and it is to be understood that the invention is not limited to the details. The details of this method for isolating  $Pa^{233}$  and  $U^{233}$  were developed by working with a number of small samples of these radioactivities formed in small bombardments, and with part of the isotopes which were obtained from 5 kg. of thorium nitrate ( $Th(NO_3)_4 \cdot 4H_2O$ ) which was bombarded in the form of an aqueous saturated solution with neutrons obtained from about 14,000 micro-ampere-hours of deuterons on beryllium. The separations were carried out before any appreciable quantity of  $Pa^{233}$  had decayed to  $U^{233}$ .

#### Example 1

The 5 kg. of neutron bombarded thorium nitrate containing  $Pa^{233} + U^{233}$  was diluted up to 26 liters with water and then made approximately 0.5 N in nitric acid. To this total solution was added about 400 grams of manganese chloride. The solution was heated and the manganese was precipitated as manganese dioxide from the hot solution by the addition of a soluble manganate or permanganate, especially an alkali manganate or permanganate such as potassium permanganate. Each precipitate of manganese dioxide was centrifuged out separately. The protoactinium is carried down with the manganese dioxide in a substantially quantitative manner under these conditions.

The combined manganese dioxide precipitates were dissolved in a mixture of hydrogen peroxide and hydrochloric acid. After decomposing the hydrogen peroxide by boiling, about 200 mg. of zirconium oxychloride were added to this solution, the zirconium was precipitated as zirconium phosphate by the addition of phosphoric acid, and the precipitate was centrifuged out separately. Zirconium phosphate carries down the protoactinium essentially quantitatively, thereby separating the latter from the relatively large amount of manganese dioxide with which it was originally associated.

It was now necessary to remove the  $Pa^{233}$  from the rather large amount of zirconium with which it was present, and to purify it from uranium and thorium. The zirconium phosphate containing protoactinium phosphate and other phosphates was brought into solution by treatment with dilute hydrofluoric acid. This step also gave a separation from thorium, which was converted to the insoluble fluoride at this point and sep-

arated. The solution was cooled with ice water and zirconium and protoactinium hydroxides were precipitated by adding dilute sodium hydroxide solution; the solution must be kept cold in this precipitation since otherwise difficulty will be experienced in redissolving the precipitated hydroxides. The hydroxide precipitate was then dissolved in nitric acid and the protoactinium was carried away from most of the zirconium by another series of manganese dioxide precipitations. Some of the zirconium comes along with the manganese dioxide precipitate in this procedure so that a further removal of the zirconium, as well as the manganese, from the protoactinium was necessary. This involved going through the above described cycle two more times, finally ending up with a small zirconium phosphate precipitate containing substantially all the protoactinium that was originally present.

This zirconium phosphate precipitate, which now contained only about 10 mg. of zirconium, was dissolved in hydrofluoric acid, and the zirconium and protoactinium then precipitated as the hydroxides as described above. This hydroxide precipitate was then converted to the corresponding nitrates by dissolving in nitric acid. Another precipitation of the zirconium phosphate (carrying the protoactinium) was then made in order to be sure that all the uranium and thorium, to amounts less than a microgram, were removed. The final zirconium phosphate was converted into zirconium sulphate by dissolving in hydrofluoric acid, precipitating the zirconium as the hydroxide, dissolving the hydroxide in sulphuric acid, and evaporating to dryness. The protoactinium accompanies the zirconium through this series of conversions.

The final zirconium sulphate (containing about 10 mg. of zirconium and the protoactinium) was dissolved in about 30 cc. of 0.33 M solution of ammonium fluoride or other alkali fluoride such as KF and the hydrogen ion concentration of the solution was adjusted until it corresponded to that of the methyl red indicator end point. The  $Pa^{233}$  was now isolated by an electrolytic procedure; in this procedure the  $Pa^{233}$  was deposited in a very thin adherent layer and was separated from the zirconium at the same time. The electrolysis chamber consisted of a clear Bakelite chamber fitted with a brass plug which screwed into the lower end and upon which rested a copper disk upon which the  $Pa^{233}$  was deposited. This copper disk served as the cathode, while a motor-driven platinum stirrer served as the anode. The electroplating was carried out for about 8 hours at about 100 milliamperes of current, applying about 15 volts across the electrolysis chamber. The  $Pa^{233}$  is plated out nearly quantitatively (about 90 percent) under these conditions. No zirconium plates out under these conditions, so that a good separation of protoactinium from zirconium is obtained by this procedure. The  $Pa^{233}$  may then be stored until it has decayed substantially to  $U^{233}$ , or it may be allowed to decay partially to  $U^{233}$  and the  $U^{233}$  separated from the  $Pa^{233}$  by any method of separating uranium from protoactinium.

By way of example, a separation of  $U^{233}$  from  $Pa^{233}$  was made by us as follows:

The thin plated film containing the  $Pa^{233}$  and  $U^{233}$  and which had aged about two months was dissolved in 6 N hydrochloric acid to which a few drops of 6 N nitric acid had been added. Since a small amount of copper was dissolved from the backing plate in this procedure this was removed by an  $H_2S$  precipitation from the acid solution. No  $Pa^{233}$  or  $U^{233}$  was carried down by the copper sulphide in this precipitation. After the removal of the  $H_2S$  and the reduction of the amount of 6 N hydrochloric acid to about 2 cc., by boiling the solution, there was added about 0.1 mg. of zirconium as zirconium oxychloride. There was then added about a hundredth of a cc. of 85 percent phosphoric acid and the precipitated zirconium phosphate was removed by centrifugation.

The major portion of the  $\text{Pa}^{233}$ , approximately 70 percent or more, was removed in this step. The yield of  $\text{Pa}^{233}$  in this precipitate is lower than that obtained when a large excess of phosphoric acid is used; however, an excess of phosphoric acid must be avoided because the acidity of the solution must be kept very low in the electrolysis procedure which follows: It is essential that less than 0.1 percent of the  $\text{Pa}^{233}$  remain with the  $\text{U}^{233}$  to avoid the simultaneous electrolytic deposition of  $\text{Pa}^{233}$  with the  $\text{U}^{233}$  and hence further separations were necessary. Further separations of the  $\text{Pa}^{233}$  from the  $\text{U}^{233}$  were effected by adding zirconium, about 0.1 mg. at a time in successive portions, to the solution. The  $\text{Pa}^{233}$  was not carried down quantitatively by the zirconium phosphate under these conditions so that it was necessary to make about 15 precipitations of zirconium phosphate, by the addition of zirconium to the phosphoric acid solution in this manner. After performing this number of precipitations, less than 0.1 percent of the  $\text{Pa}^{233}$  remained in the solution. Practically all of the  $\text{U}^{233}$  remains in solution in this procedure; however, it should be emphasized that in order for this to be the case it is necessary that the  $\text{Pa}^{233}$  be removed with small successive portions of zirconium phosphate in the manner which has been described.

The volume of the solution was then reduced, by evaporation, to a volume of about 0.1 cc. To this solution, which contained about 0.10 cc. of 6 N hydrochloric acid and of the order of 0.001 cc. of 85 percent phosphoric acid, there was added 0.02 cc. of glacial acetic acid and the solution was diluted by the addition of 5 cc. of water. This solution was placed in an electrolysis chamber which consisted of a clear Bakelite chamber fitted with a brass plug that screwed into the lower end and upon which rested a platinum foil that the  $\text{U}^{233}$  was to be deposited upon. The electroplating was carried out for about 8 hours at about 90 milliamperes of current applying about 8 volts across the electrolysis chamber (the actual electrode potential for  $\text{U}^{233}$  is not known). The  $\text{U}^{233}$  is plated out nearly quantitatively (greater than 90 percent) under these conditions and the plate usually appears as a well adhering film of pure  $\text{U}^{233}$  (probably in the form of the trifaoctaoxide,  $\text{U}_3^{233}\text{O}_8$ ) together with a small amount of organic matter which can be burned off the plate. It should be emphasized that in order for the uranium to be quantitatively deposited the acidity of the solution must be kept very low as described above. (In addition, it may be pointed out that this electrolysis may be performed from an 0.3 M ammonium fluoride solution, with approximately the same yields, and in some experiments we have used this procedure.) The weight of the  $\text{U}^{233}$  sample prepared in the manner outlined above, as determined from its alpha activity and from the half-life of  $\text{U}^{233}$  ( $1.2 \times 10^5$  years), was found to be 3.8 micrograms.

The preferred method for separating protoactinium from zirconium is the electrolysis from ammonium fluoride solution, described above, wherein microgram (or less) quantities of protoactinium are deposited while as much as 10 mg. of zirconium remain in solution. Another method is the precipitation of the protoactinium with manganese dioxide. In this procedure a certain amount of zirconium is also carried along with the manganese dioxide; this small amount of zirconium can be removed from the manganese by precipitation as zirconium phosphate which carries the protoactinium with it. After dissolving the zirconium-protoactinium phosphate in dilute hydrofluoric acid solution, the protoactinium can be removed by another manganese dioxide precipitation and this cycle may be repeated as often as is necessary in order to remove practically all the zirconium from the protoactinium. In a third method the protoactinium is removed with lanthanum oxalate by making a number of successive precipitations of lanthanum oxalate from a dilute hydrochloric acid solution; six or eight precipita-

tions will carry about 80 percent of the protoactinium, while carrying a negligible amount of the zirconium, which remains in solution as a complex oxalate. (The protoactinium can then be removed from the lanthanum oxalate by dissolving the latter in hydrochloric acid and precipitating a very small amount of zirconium phosphate from this solution.) A fourth method involves the fractional precipitation of zirconium iodate. If there is added to a 1 to 6 N  $\text{HCl}$  or  $\text{HNO}_3$  solution, containing a mixture of zirconium and protoactinium, a small amount of sodium iodate, sufficient to precipitate only a small fraction of the zirconium as zirconium iodate, it is found that the protoactinium concentrates to a large extent in this first fraction. This precipitate can be dissolved in concentrated hydrochloric acid and again a partial precipitation of zirconium iodate performed; in each cycle a large concentration of protoactinium is obtained. By removing several zirconium iodate precipitates in each cycle, the protoactinium can be brought along quantitatively. Finally, a solution containing a salt of zirconium and  $\text{Pa}^{233}$  in solution can be made 6 to 10 N in hydrochloric acid and subjected to fractional crystallization for the separation of zirconium oxychloride in crystalline form, whereupon the protoactinium concentrates in the mother liquor.

#### Example 2

A solution containing 300 grams per liter of neutron irradiated thorium nitrate tetrahydrate and an acidity of 1 N nitric acid was prepared. This solution contained about 2 parts by weight of  $\text{Pa}^{233} + \text{U}^{233}$  per million parts of thorium. Manganese nitrate was added in excess of the amount required to form 1.1 grams per liter of  $\text{MnO}_2$  and sufficient potassium permanganate was added to precipitate a total of 1.1 grams per liter of  $\text{MnO}_2$  in two approximately equal portions and the  $\text{MnO}_2$  containing the  $\text{Pa}^{233}$  was recovered.

The  $\text{MnO}_2$  was dissolved in a mixture of nitric acid and hydrogen peroxide and the solution was boiled to decompose excess peroxide and diluted to about 20 grams per liter of manganese nitrate per liter and an acidity of 1 normal nitric acid.  $\text{MnO}_2$  was again precipitated in the proportion equivalent to about 10 percent by weight of the manganese nitrate in solution. The process of dissolving and precipitating  $\text{MnO}_2$  was repeated several times and the  $\text{MnO}_2$  finally obtained was dissolved in nitric acid and concentrated to 4 M manganese ion. Thereupon the aqueous solution was permitted to age until a major portion of the  $\text{Pa}^{233}$  in solution had decayed to  $\text{U}^{233}$ . This  $\text{U}^{233}$  was then extracted from the solution with ether.

In accordance with a further modification of the invention, other methods may be used for recovering a  $\text{Pa}^{233}$  concentrate which may be aged to form  $\text{U}^{233}$ . For example an aqueous solution of neutron irradiated thorium such as a nitric acid solution may be treated with hydrogen fluoride substantially in excess of that required to form thorium fluoride. In such a case the thorium precipitates leaving  $\text{Pa}^{233}$  in solution. This  $\text{Pa}^{233}$  may then be treated to recover a  $\text{Pa}^{233}$  by convenient means such as we have heretofore described.

Moreover the  $\text{Pa}^{233}$  may be recovered or removed as a concentrate from a nitric acid acidified solution by precipitation of about 10-20 percent by weight of the thorium as thorium iodate which carries down the  $\text{Pa}$  in the solution. For example a thorium nitrate solution having a nitric acid normality of about 4 may be treated with sufficient potassium iodate to precipitate 10-20 percent of the thorium as thorium iodate in order to remove the  $\text{Pa}$ . This precipitate may be redissolved and retreated in order to increase the  $\text{Pa}$  concentration if desired.

In the specification and claims, wherever reference is made to the presence or the addition of phosphoric acid or a phosphate, unless otherwise indicated by the context, it is to be understood that the reference is to ortho-phosphoric acid or its salts.

By the above methods of separating  $\text{Pa}^{233}$  and  $\text{U}^{233}$  from foreign products we are able to obtain compositions composed largely or entirely of  $\text{U}^{233}$  compounds, which are substantially free from fission products. The  $\text{U}^{233}$  metal may be produced from suitable compounds thereof by calcium reduction or any of the other known methods for producing uranium metal from compounds of uranium.

$\text{U}^{233}$  metal or compounds of  $\text{U}^{233}$  may be shaped into the form of spheres, cylinders, blocks or the like by known methods of shaping uranium metal and compounds. Such shaped articles of manufacture may be used as a source of nuclear power as described in our copending application, Serial No. 565,990, filed November 30, 1944.

While there has been described certain embodiments of our invention, it is to be understood that it is capable of many modifications. Changes, therefore, may be made without departing from the spirit and scope of the invention as described in the appended claims, in which it is the intention to claim all novelty in the invention as broadly as possible.

We claim:

1. The method of separating  $\text{Pa}^{233}$  from foreign products present in neutron irradiated thorium which comprises forming a solution of neutron irradiated thorium and a manganous salt, then adding a substance selected from the class consisting of soluble manganates and permanganates to precipitate manganese as manganese dioxide whereby protoactinium is carried down with the manganese dioxide.

2. The method of separating  $\text{Pa}^{233}$  from foreign products present in neutron irradiated thorium which comprises forming a solution of neutron irradiated thorium and a manganous salt, then adding potassium permanganate to precipitate the manganese as manganese dioxide whereby protoactinium is carried down with the manganese dioxide; dissolving the precipitate, adding a soluble zirconium salt, and adding phosphate ion to precipitate zirconium phosphate whereby protoactinium is carried down with the zirconium phosphate.

3. The method as in claim 1, wherein potassium permanganate is employed as the substance for precipitating manganese dioxide.

4. A method of recovering  $\text{Pa}^{233}$  which comprises form-

ing a solution of neutron irradiated thorium containing  $\text{Pa}^{233}$  and contacting the solution with manganese dioxide which removes  $\text{Pa}^{233}$  from the solution.

5. The method of separating protactinium from uranium and thorium, which comprises forming a solution containing ions of said elements and a manganous salt, then adding a substance selected from the class consisting of soluble manganates and permanganates to precipitate manganese as manganese dioxide whereby protoactinium values are carried down with the manganese dioxide.

10 6. The method of separating protoactinium from uranium and thorium, which comprises forming a solution containing ions of said elements and a manganous salt, then adding potassium permanganate to precipitate the manganese as manganese dioxide whereby protoactinium is carried down with the manganese dioxide, dissolving the precipitate, adding a soluble zirconium salt, and adding phosphate ion to precipitate zirconium phosphate whereby protoactinium is carried down with the zirconium phosphate.

15 7. A method of separating  $\text{Pa}^{233}$  from zirconium which comprises precipitating  $\text{Pa}^{233}$  with a carrier precipitate of manganese dioxide from an aqueous solution containing zirconium and  $\text{Pa}^{233}$ .

20 8. A method of separating protoactinium values from zirconium which comprises precipitating protoactinium values with a carrier precipitate of manganese dioxide from an aqueous solution containing zirconium and protoactinium.

#### References Cited in the file of this patent

#### UNITED STATES PATENTS

35 1,120,551 Schwerin ----- Dec. 8, 1914  
2,206,634 Fermi et al. ----- July 2, 1940

#### OTHER REFERENCES

Friend: Textbook of Inorganic Chemistry, vol. 7, part 3, page 303 (1926), published by Charles Griffin & Co., Ltd., London.

Piggot: Physical Review, 2nd series, vol. 43, pages 51-59 (1933); pages 55 and 57 particularly relied on.

Nature, June 16, 1934, page 899.

Turner: Physical Review, vol. 57, page 157 (1940).